

Patented Oct. 24, 1922.

1,432,742

# UNITED STATES PATENT OFFICE.

FREDERICK JAMES COMMINS, OF LONDON, ENGLAND.

## TREATING PITCH.

No Drawing.

Application filed December 27, 1920. Serial No. 433,436.

To all whom it may concern:

Be it known that I, FREDERICK JAMES COMMINS, a subject of the King of Great Britain and Ireland, residing at London, England, have invented certain new and useful Improvements in Treating Pitch, of which the following is a specification.

The object of this invention is the production of a pitch in an extremely fine state of division.

The invention consists in grinding the pitch in the presence of a solution of a peptonizing agent in order that it can be obtained in a very finely divided state in which form it can be readily and uniformly distributed with other materials in the presence of a suitable liquid.

Suitable peptonizing agents are: casein dissolved in a dilute solution of alkali or a solution of sodium rosinate in water.

When the pitch is ground in the presence of these substances, the fine particles produced are prevented from adhering together again or are deflocculated and the resulting product can be readily dispersed in water. The fine particles only deposit very slowly or not at all and are in a semi colloidal state.

According to one mode of carrying out the invention the coarsely ground pitch is treated in a ball mill with an amount of water equal in weight to the pitch taken, and in which is dissolved resin soap, the latter acting as a peptonizing agent. The amount of peptonizing agent taken should be approximately equal to 2% of the weight of the pitch. The whole is ground in the mill till the desired degree of dispersion is obtained, say from one to six hours.

One application of the invention is in the manufacture of cellulose fibre compositions of which pitch, in a very finely divided state and uniformly distributed, forms one of the components, the peptonized or deflocculated pitch being added to a cellulose pulp. The effect of the mixing of the peptonized pitch with the cellulose fibre is to withdraw the former from its state of semi solution in the water which can be drained away substantially free from pitch.

In the resulting composition the pitch, in a very finely divided state, is uniformly distributed in a manner hitherto impossible or extremely difficult to obtain.

I claim:

1. The method of treating pitch to bring

it into an extremely fine state of division, consisting in grinding the pitch in a solution of a peptonizing agent, with said solution in sufficient quantity to produce a resultant mass of liquid consistency in the nature of a pitch cream. 60

2. The method of treating pitch to bring it into an extremely fine state of division, consisting in grinding the pitch in a solution of resinous material, with said solution in sufficient quantity to produce a resultant mass of liquid consistency in the nature of a pitch cream. 65

3. The method of treating pitch to bring it into an extremely fine state of division, consisting in grinding the pitch in a solution of a resin soap, with said solution in sufficient quantity to produce a resultant mass of liquid consistency in the nature of a pitch cream. 70

4. The method of treating pitch to bring it into an extremely fine state of division, consisting in grinding the pitch in a solution of a sodium rosinate in water, with said solution in sufficient quantity to produce a resultant mass of liquid consistency in the nature of a pitch cream. 75

5. The method of treating pitch to bring it into an extremely finely divided state, consisting in subjecting coarsely ground pitch to a grinding action in a ball mill, in a solution of a peptonizing agent, with such solution in sufficient quantity to produce a resultant mass of liquid consistency in the nature of a pitch cream. 80

6. The method of treating pitch to bring it into an extremely finely divided state, consisting in subjecting coarsely ground pitch with water in which a peptonizing agent is dissolved to a grinding action in a ball mill, with the water solution of the peptonizing agent in sufficient quantity to produce a resultant mass of liquid consistency in the nature of a cream. 85

7. A method of treating pitch to bring it into an extremely finely divided state consisting in subjecting coarsely ground pitch to a grinding action in a ball mill with a water solution of a peptonizing agent, the amount of water being equal in weight to the pitch, and the amount of peptonizing agent being equal in weight approximately to two per cent of the weight of the pitch. 90

8. A method of obtaining pitch in an extremely fine state of division consisting in treating coarsely ground pitch in a ball mill. 110

with an amount of water equal in weight to the pitch, having dissolved therein a resin soap in amount equal approximately to two per cent of the weight of the pitch, the ball mill treatment being continued until the desired degree of dispersion is obtained.

9. A finely divided pitch obtained by

grinding pitch in the presence of a solution of a peptonizing agent the fine particles being deflocculated and in a semi colloidal state.

In testimony whereof I have signed my name to this specification.

FREDERICK JAMES COMMINS.